

## 1

3,726,798

### HYDRAULIC FLUID CONTAINING BASIC ZINC CARBOXYLATES

Howard Bernard Silver, Hinchley Wood, England, assignor to The British Petroleum Company Limited, London, England

No Drawing. Filed Apr. 14, 1971, Ser. No. 134,077  
Claims priority, application Great Britain, Apr. 28, 1970,  
20,320/70

Int. Cl. C09k 3/00

U.S. Cl. 252—75

8 Claims

#### ABSTRACT OF THE DISCLOSURE

Hydraulic fluids containing novel complexes of zinc dihydrocarbyl dithiophosphates and basic zinc carboxylates are non-corrosive to silver.

This invention relates to an improved hydraulic fluid.

Hydraulic fluids are fluids intended for use in hydraulic fluid power systems.

A useful source of information on this subject is the book "Introduction to Hydraulic Fluids" by Roger E. Hatton, published by Reinhold Publishing Corporation, New York, in 1962. Hatton defines a hydraulic fluid power system as a means of power transmission in which a relatively incompressible fluid is used as a power transmitting medium and states that the primary purpose of a hydraulic system is the transfer of energy from one location to another and the conversion of this energy to useful work. He divides the functions of a hydraulic system into the aspects of (a) generation, (b) utilisation, (c) transmission and (d) control of fluid power. Hydraulic power is usually generated by special pumps.

Amongst the many desirable physical and chemical properties of hydraulic fluids are some which unfortunately are conflicting in their requirements. Good load carrying ability is desirable and in order to achieve this it is common practice to add load carrying additives, frequently reactive sulphur compounds such as sulphides, phosphosulphurised hydrocarbons and, in particular, zinc dihydrocarbyl dithiophosphates. The latter are very useful additives because in addition to their load carrying properties they also act as antioxidants.

It is necessary that hydraulic fluids should be non-corrosive towards metallic surfaces with which they come into contact.

Hydraulic pumps may contain slipper pads plated with silver to reduce wear and unfortunately these are attacked by reactive sulphur containing compounds.

Thus it is possible to obtain hydraulic fluids which have satisfactory load-carrying properties but which are corrosive to silver.

It is also possible to obtain hydraulic fluids which are non-corrosive to silver but which have unsatisfactory load carrying properties.

The two conflicting requirements of adequate load-carrying performance and non-corrosivity to silver pose a difficult problem.

British patent specification 959,115 discloses a new class of zinc dithiophosphate additives which are stated to be non-corrosive to silver. The class comprises two types of zinc dithiophosphate salts, viz., (1) normal size bis-(aryl)-dithiophosphates and (2) normal zinc bis-(alkyl)-dithiophosphates prepared from so-called neo- or hindered-type alcohols, i.e. alcohols in which the carbon atom adjacent to the carbon atom attached to the hydroxyl group is completely substituted with alkyl groups.

I have now discovered novel complexes, the nature of which I am not certain, of zinc dihydrocarbyl dithiophosphates and basic zinc carboxylates which, when added to hydraulic fluids, are substantially non-corrosive to silver.

## 2

Thus according to the present invention there is provided a complex of (A) a zinc dihydrocarbyl dithiophosphate of formula



wherein  $R^1$ — $R^4$  are alkyl groups containing 2 to 18 carbon atoms, aryl groups containing 6—12 carbon atoms or alkyl groups containing 7—15 carbon atoms, with (B) a basic zinc carboxylate of formula  $(R^5COO)_6Zn_4O$  wherein  $R^5$  is an alkyl, cycloalkyl, aryl, aralkyl or alkaryl group preferably having not more than 24 carbon atoms, the compound having a tetrahedral structure with the 4 zinc atoms at the corners, the oxygen atom in the centre and the 6 carboxylate groups arranged along the sides. Most suitably  $R$  is an alkyl group having up to 18 carbon atoms.

Suitable zinc dihydrocarbyl dithiophosphates include zinc di-n-butyl dithiophosphate, zinc di-n-pentyl dithiophosphate, zinc di-isohexyldithiophosphate, zinc di-4-methylpent-2-yl dithiophosphate, zinc di-p-octylphenyl dithiophosphate and zinc di-isohexylophenyldithiophosphate.

Suitable basic zinc carboxylates are described in British patent specification 1,142,195 and include basic zinc octanoate, basic zinc 2-ethylhexanoate, basic zinc versatate and basic zinc oleate.

The complex may simply be prepared by mixing component (A) with component (B). If the complex is to be used as an additive then the components may be mixed before or after being added to the base stock.

The simple method of preparation contrasts with the method employed to prepare the zinc carboxylate co-ordinated-zinc dithiophosphate salts of British patent specification 959,115. British patent specification 959,115 discloses a method in which the zinc carboxylate and zinc dithiophosphate are heated in the presence of water and a hydrocarbon solvent and water is distilled off to obtain a solution of the complex salt.

It is a further advantage of my complex salt that water is not used during its preparation. Water tends to hydrolyse irreversibly complex zinc salts.

The components are suitably mixed in a ratio in the range 1 to 5, preferably 1 to 1.

Zinc dihydrocarbyl dithiophosphates with various hydrocarbyl radicals are readily available from additive manufacturers under a variety of trade names.

Basic carboxylates may be prepared by reacting one mole of proportion of zinc oxide with 1.5 moles of proportions of an acid of formula  $R^5COOH$ , wherein  $R^5$  is as previously defined. Details of the preparation of these compounds are given in British patent specification 1,142,195.

As stated above, the complexes are very suitable for use as load-carrying additives to hydraulic fluids which are substantially non-corrosive to silver.

Thus according to a further feature of the present invention there is provided a hydraulic fluid comprising a major proportion of a base oil and a minor proportion of a complex as hereinbefore described.

Suitably the fluid contains 0.1 to 5%, preferably 0.5 to 2% by weight of the complex.

The base stock may be a mineral oil or a synthetic material.

Suitable mineral oils are paraffinic oils of viscosity in the range 2.0 to 20 cst. at 98.8° C.

The preferred mineral oil is characterized by a viscosity of 5 cst. at 98.8° C.

Suitable synthetic bases include esters of phosphorus containing acids, e.g., triaryl phosphates, silicate esters, halogenated hydrocarbons, e.g. chlorinated diphenyl, esters of organic acids with alcohols or phenols, and polyalkylene glycols.

If the hydraulic fluid is based on a mineral oil, a pour point depressant may be necessary. Suitable pour point depressants include n-alkylated aromatic compounds. They are conveniently used in amount 0.1 to 2% by wt.

It is also very desirable that the hydraulic fluid should contain a small amount e.g., 0.01-0.5% by weight of a rust inhibitor. Suitable rust inhibitors include alkenyl succinic acids, alkyl mercapto acidic acids and alkaryloxy acetic acids.

Other additives which may be used to advantage in specific uses of the hydraulic oil include viscosity index improvers, e.g., polyisobutenes, polyalkylmethacrylates and polyalkylstyrenes, and antifoam agents, e.g., silicone fluids.

The invention is illustrated by the following examples.

RESULTS OF EMD SILVER CORROSION TEST ON BLENDS OF ZINC DIARYL DITHIOPHOSPHATE (OLOA 260) WITH AND WITHOUT ZINC CARBOXYLATES

| Example                                              | 1               | 2            | 3                       |
|------------------------------------------------------|-----------------|--------------|-------------------------|
| Oloa 260, percent                                    | 1.0             | 1.0          | 1.0                     |
| Plexol 150, percent                                  | 0.4             | 0.4          | 0.4                     |
| Zinc octanoate, percent                              |                 | 1.0          |                         |
| Basic zinc octanoate, percent                        |                 |              | 1.0                     |
| Base oil, percent                                    | 98.6            | 97.6         | 97.6                    |
| Appearance of silver plate after 72 hours            | Grey-black film | Multi-colour | Dull grey/brown tarnish |
| Weight change, mg.                                   | -112, -114      | -2.4, -2.8   | -0.1, -0.1              |
| Four ball anti-wear test                             | 0.29            | 0.58         | 0.36                    |
| Wear scar diameter after 1 hr. with 15 kg. load, mm. |                 |              |                         |

NOTE.—Oloa 260 is a zinc diaryl dithiophosphate sold by Orobis Ltd. Plexol 150 is an alkylated naphthene wax pour point depressant sold by Rohm & Haas. Base oil is a solvent refined paraffinic mineral oil with a viscosity of 5.2 est. at 98.8° C.

The EMD silver corrosion test is a test developed by the Electro Motive Division of General Motors Corporation. Details of this test are given in the previously mentioned 959,115.

EFFECT OF ZINC CARBOXYLATES ON ZINC DIALKYL DITHIOPHOSPHATES

| Example                                                                                  | 4                                         | 5                                                | 6                              | 7                                            | 8                                           | 9                         |
|------------------------------------------------------------------------------------------|-------------------------------------------|--------------------------------------------------|--------------------------------|----------------------------------------------|---------------------------------------------|---------------------------|
| Plexol 150                                                                               | 0.4                                       | 0.4                                              | 0.4                            | 0.4                                          | 0.4                                         | 0.4                       |
| Anglamol 75                                                                              | 1.0                                       |                                                  | 1.0                            | 1.0                                          | 1.0                                         |                           |
| Lubrizol 1360                                                                            |                                           |                                                  | 1.0                            |                                              |                                             |                           |
| Normal zinc octoate                                                                      |                                           |                                                  | 1.0                            |                                              |                                             |                           |
| Basic zinc octoate                                                                       |                                           |                                                  |                                | 1.0                                          | 2.0                                         | 1.0                       |
| Base oil                                                                                 | 98.6                                      | 98.6                                             | 97.6                           | 97.6                                         | 96.6                                        | 97.6                      |
| EMD silver corrosion test. Appearance of silver plate and wt. loss (mg.) after 72 hours. | Black with green/blue tarnish (240; 229). | Dark brown tarnish with black deposits (33; 40). | Black flaky deposits (39; 52). | Blue/grey tarnish with flaky solid (22; 14). | Slight tarnish almost unchanged (1.8; 1.7). | Light tarnish (2.2; 2.3). |
| Four ball wear test 15 kg./1 h./ambient (wear scar diameter) mm.                         | 0.28                                      | 0.26                                             |                                |                                              | 0.26                                        | 0.31                      |

NOTE.—Anglamol 75 is a rust inhibiting, anti-wear, anti-oxidant and anti-corrosive package sold by the Lubrizol Corporation. It contains zinc dialkyl dithiophosphate. Lubrizol

basic zinc carboxylate of formula  $(R^5COO)_6Zn_4O$  where in  $R^5$  is an alkyl, cycloalkyl, aryl, aralkyl or alkaryl group preferably having not more than 24 carbon atoms, the compound having a tetrahedral structure with the 4 zinc atoms at the corners, the oxygen atom in the centre and the 6 carboxylate groups arranged along the sides, the molar ratio of component (A) to component (B) being in the range of 1:1 to 1:5.

5 2. A hydraulic fluid according to claim 1 which contains 0.5 to 2% by weight of the complex.

3. A hydraulic fluid according to claim 1 in which the mineral oil is a paraffinic oil of viscosity in the range 2 to 20 centistokes at 98.8° C.

10 4. A hydraulic fluid according to claim 1 in which the mineral oil has a viscosity of 5 centistokes at 98.8° C.

5. The hydraulic fluid as claimed in claim 1 in which  $R^5$  is an alkyl group having up to 18 carbon atoms.

20 6. The hydraulic fluid as claimed in claim 1 wherein said zinc dihydrocarbyl dithiophosphate of said complex is zinc di-n-butyl dithiophosphate, zinc di-n-pentyl dithiophosphate, zinc di-isohexyl dithiophosphate, zinc di-4-methylpent-2-yl dithiophosphate, zinc di-p-octylphenyl dithiophosphate or zinc di-isohexylphenyl dithiophosphate.

25 7. The hydraulic fluid as claimed in claim 1 wherein said basic zinc carboxylate of said complex is basic zinc octanoate, basic zinc 2-ethylhexanoate, basic zinc versatate or basic zinc oleate.

30 8. The hydraulic fluid as claimed in claim 1 wherein the molar ratio of (A) to (B) is 1:1 in said complex.

1360 is a similar composition sold by the Lubrizol Corporation. The base oil is as previously described for Examples 1-3.

It should be noted that Examples 1, 2, 4, 5 and 6 are provided for purposes of comparison only and are not in accordance with the present invention.

I claim:

1. A hydraulic fluid consisting essentially of a mineral oil and from 0.1% to 5% by weight of a complex of (A) a zinc dihydrocarbyl dithiophosphate of formula



wherein  $R^1-R^4$  are alkyl groups containing 2 to 18 carbon atoms, aryl groups containing 6-12 carbon atoms or alkaryl groups containing 7-15 carbon atoms, with (B) a

References Cited

UNITED STATES PATENTS

3,328,335 6/1967 Jolie ----- 252—32.75  
3,523,081 8/1970 Braid ----- 252—75 X

LEON D. ROSDOL, Primary Examiner

65 H. A. PITLICK, Assistant Examiner

U.S. Cl. X.R.

252—32.7 E, 76; 260—429.9